# EUROPEAN PATENT SPECIFICATION

(11) **EP 2 646 582 B1**
(45) Date of publication and mention of the grant of the patent: **30.10.2019**
(21) Application number: 11815448.3
(22) Date of filing: 01.12.2011
(51) Int. Cl.: C21D 1/18, C21D 8/02, C22C 38/42, C22C 38/44, C22C 38/50

(54) **ULTRA HIGH-STRENGTH STRUCTURAL STEEL AND METHOD FOR PRODUCING ULTRA HIGH-STRENGTH STRUCTURAL STEEL**
ULTRAHOCHFESTER BAUSTAHL UND VERFAHREN ZUR HERSTELLUNG DES ULTRAHOCHFESTEN BAUSTAHLS
ACIER STRUCTUREL À ULTRA-HAUTE RÉSISTANCE ET PROCÉDÉ DE PRODUCTION D'UN ACIER STRUCTUREL À ULTRA-HAUTE RÉSISTANCE

(30) Priority: 02.12.2010 FI 20106275
(43) Date of publication of application: 09.10.2013
(73) Proprietor: Rautaruukki Oyj, 00620 Helsinki (FI)
(72) Inventor: LIIMATAINEN, Tommi, FI-92130 Raahe (FI)
(74) Representative: Valea AB
(86) International application number: PCT/FI2011/051066
(87) International publication number: WO 2012/072884

(56) References cited:
- GB-A- 1 161 056
- US-A- 4 572 748
- US-A- 4 946 516
- US-A1- 2004 031 544
- US-B1- 6 245 290
- SPIEKERMANN P: "Legierungen - ein besonderes patentrechtliches Problem?", MITTEILUNGEN DER DEUTSCHEN PATENTANWAELTE, HEYMANN, KOLN, DE, vol. 34, 1 January 1993 (1993-01-01), pages 178-190, XP002152326, ISSN: 0026-6884

## Description

### Background of the invention

The invention relates to an ultra high-strength structural steel, which is produced by hot-rolling as a sheet-like steel product.

More specifically, the invention relates to an ultra high-strength structural steel according to the preamble of claim 1 and a method for producing an ultra high-strength structural steel according to the preamble of claim 11. By an ultra high-strength structural steel is meant steel, whose yield strength R_{p0.2} is at least 960MPa and yield ratio (R_{p0.2}/ Rₘ) is more than 0.7, which is typical especially of direct quenched structural steels.

The invention relates to production of an ultra high-strength structural steel, whose composition, as percentages by weight, is recited in claim 1.

The invention also relates especially to an ultra high-strength structural steel, whose composition comprises above said elements, wherein, in addition to high strength, the ultra high-strength structural steel also has excellent weldability by possessing excellent impact toughness properties in the heat affected zone of the weld.

Structural steels are used in construction and transportation equipment industries, in which the trend is to use stronger steels to achieve lighter structures. In this case, steel structures can be lightened, the load-bearing capacity of machines and devices improved and energy consumption decreased. An attempt is made to provide a steel that is as strong as possible, but, as strength increases, usability properties, such as weldability and flangeability as well as other important properties, such as elongation and impact toughness can weaken, as is known. Especially, in such strong steels, the risk related to the hydrogen cracking of welding is great and fracture behaviour is sometimes unsure, which makes the work of the structural engineer and the calculator of strength problematic. In the heat affected zone (HAZ) of the weld, there also cannot be during welding any significant softening, or at least the width of the softened zone should remain as narrow as possible, in order that the strength of the welded joint remains good, i.e. as close as possible to the strength of the base metal. Other mechanical properties of the heat affected zone of the weld, such as elongation and especially impact toughness, should also remain as good as possible, in order that the design work of practical structures remain sensible and as simple as possible and the functionality of the structures in practise is assured.

As is known, also the heat input must be significantly limited when welding high and ultra high-strength steels, which can cause an unfavourable form of weld bead for fracture toughness and fatigue resistance, because, at a low heat input, the junction point of the weld metal and base metal does not form smoothly as easily as at a higher heat input. Limitation of the heat input also weakens the productivity of welding work, adding expenses.

Moreover, structural steels must sometimes be weather-resistant, wherein the steel does not necessarily need to be coated because an tight oxide layer forms on the surface of the steel, which significantly slows down the progress of corrosion. In demanding sites, the steel must withstand, in addition to normal climatic stress, also the sodium chloride NaCl contained in a maritime climate, wherein ultra high-strength structural steel can excellently be used also in ship and harbour structures even without coating. Also when coated, the durability of the paint surface of weather-resistant steel in local damage points of the surface is better, because the progress of rust below the paint surface slows down. Especially by ultra high-strength structural steels, the attempt is for the smallest material thicknesses possible and, therefore, assurance against corrosion damages is further emphasized.

Known is i.a. an ultra high-strength hot-rolled structural steel, the composition of which contains, as percentages by weight, typically C: 0.095 %, Si: 0.20 %, Mn: 1.0 %, Cu: 0.4 %, Cr: 1 %, Ni: 0.20 %, and Ti: 0.03 % as well as iron and unavoidable impurities. The steel in question is produced as having a yield strength greater than 960MPa, but the impact toughness of its base metal is only moderate and the steel in question does not withstand the stress of saltwater very well. Likewise, during welding, the heat affected zone of the base metal softens significantly and over a relatively wide zone, wherein the load-bearing capacity of the weld seam, such as strength and impact toughness, weakens during typical welding significantly in comparison to the load-bearing capacity of the base metal.

From KR950004775 B1 is known a method for producing a steel having a yield strength of approximately 150KSI ·1034MPa), in which method a steel of composition C: < 0.12 %, Mn: 0.6 - 0.9 %, Si: 0.2 - 0.35 %, Ni: 4.75 - 5.25 %, Cr: 0.4 - 0.7 %, Mo: 0.3 - 0.65 %, V: 0.05 - 0.10 %, P: < 0.01 %, and S < 0.015 %, the rest being iron and unavoidable impurities, is quenched from the hot-rolling process and, thereafter, temper-treated. However, the problem with this known steel is that the steel is not particularly weather-resistant, because into it was not alloyed copper Cu and also simultaneously just a small amount of chromium Cr. Solution hardening by using nickel Ni without copper Cu leads to excessively high Ni-contents, which is disadvantageous i.e. on the part of alloying element expenses. If the steel is further tempered after direct quenching, this steel has no copper Cu to precipitate, which would further increase the strength of the steel. This known steel is also not particularly weldable, because into it has not been alloyed titanium Ti to prevent grain formation at a high heat input, wherein, due to small welding energies, it is difficult to get the junction point of the weld bead and the base metal smooth, wherein a tough and strong joint is difficult to achieve.

US 4,572,748 discloses a steel plate having a high tensile strength which is manufactured from a steel consisting essentially of 0.04-0.16% by weight of C, 0.02-0.50% by weight of Si, 0.4-1.2% by weight of Mn, 0.2-5.0% by weight of Ni, 0.2-1.5% by weight of Cr, 0.2-1.0% by weight of Mo, 0.01-0.10% by weight of acid soluble Al, 0.03-0.15% by weight of one or more of V, Ti and Nb, 0.015% or less by weight of P, 0.006% or less by weight of S and the balance of iron and inherent impurities. The steel is heated to a temperature above a temperature at which carbo-nitrides of V and Nb, and carbides of Ti become complete solid solution state, rolled with total reduction of 40% or more below 950°C, quenched by simultaneous cooling immediately after completion of the rolling from a temperature above (A₃-50) DEG C. and tempered at a temperature lower than A_{c1} temperature. The density of cooling water (W) for the quenching is detemined by the following equation (I) or (II) in accordance with the plate thickness (t): (I) for the plate over 40 mm, thickness W=0.7 to 1.5 m³/min·m2 and (II) for the plate over 25 mm and under 40 mm, thickness W=0.7 to (8.5-0.1 t)/3 m³/min·m2.

US 4,946,516 concerns a process for producing steel possessing a high level of toughness and strength free of anisotropy and having good resistance to stress corrosion cracking in seawater conditions. The process comprises the steps of: preparing a steel slab comprised of 0.02 to 0.10 wt % C, 0.50 wt % or less Si, 0.4 to 1.5 wt % Mn, 1.0 to 8.0 wt % Ni, 0.1 to 1.5 wt % Mo, 0.8 wt % or less Cr, 0.01 to 0.08 wt % sol. Al, with the balance of Fe and unavoidable impurities; heating the slab to a temperature of from 1000°C to 1250°C; hot rolling the steel at a reduction rate of 20 to 60% at an austenite recrystallization temperature region and then at a reduction rate of 30 to 70% at an austenite non-recrystallization temperature region and finishing the rolling at a temperature of 650°C or higher; quenching the steel by initiating water cooling at a temperature at or above the Ar₃ point thereof and terminating the water cooling at a temperature of 150°C or lower; quenching the steel after reheating the steel to a temperature between the Ac₃ point and the Ac₃ point+100°C thereof; and tempering the steel at a temperature at or below the A_{c1} point thereof.

The combination of excellent strength and impact toughness of known ultra high-strength steels, achieved by thermo-mechanical rolling and direct quenching, weakens in the HAZ due to the heat cycle caused by welding.

Thus, the problem of known solutions is especially that there is not known an ultra high-strength hot-rolled structural steel, in which, at the same time along with high HAZ impact toughness and weather resistance of the base metal, high strength is achieved.

### Brief description of the invention

The object of this invention is to solve the problems of known art and to provide an excellent ultra high-strength structural steel, wherein the impact toughness of the HAZ of a weld joint provided in this steel is excellent. In this case, the steel can be used in welded applications requiring impact toughness, such as in welded boom structures.

The invention provides an ultra high-strength structural steel, wherein the impact toughness of the HAZ of a weld provided in this steel, as measured transversely in relation to the direction of rolling at a temperature of -40°C, is more than 34 J/ cm², i.e. expressed differently $Charpy V - 40 ° C T \left(FL, ICHAZ, CGHAZ\right) > 34 J / {cm}^{2}$

The second object of the invention is to provide a new method for producing an ultra high-strength structural steel from a steel, whose composition comprises said element contents.

To implement this, an ultra high-strength structural steel according to the invention is characterized by that what is said in the characterizing part of claim 1.

A method according to the invention is characterized by that which is said in the characterizing part of claim 11.

Advantageous embodiments of the invention are presented in the independent claims as well as in the description.

The objects of the invention are achieved by alloying the composition of the steel according to the invention and, preferably but not necessarily, by direct quenching the steel having the alloyed composition after hot-rolling. In other words, the present invention is implemented, preferably but not necessarily, by using a unique combination of the composition of the steel and direct quenching.

According to the invention, it is surprisingly found that by said composition and, preferably but not necessarily, by direct quenching a steel according to said composition, an ultra high-strength steel is achieved possessing, at the same time, good HAZ impact toughness properties and having the excellent weather resistance and weldability properties. Specifically, in the invention, it is surprisingly found that a highly nickel- and/or copper-alloyed as well as with, at the most, a small amount of titanium-alloyed steel achieves an ultra high-strength steel, whose base metal and weld HAZ strength and impact toughness are at an excellent level.

The greatest advantages of an ultra high-strength structural steel according to the invention are that it has ultra-high strength combined with good impact toughness and it can excellently be welded such that the mechanical properties of the HAZ are excellent. Welding can even be done without preheating. During welding, the problems relating to hydrogen cracking can be avoided and thus can be used, for such a strong direct quenched structural steel, reasonably great heat input, wherein the load-bearing capacity of the weld remains at an excellent level and the efficiency of welding work can be kept high. Further, a structural steel according to the invention has good properties relating to fracture toughness, which is advantageous especially in extreme stress situations. As a significant advantage is the high impact toughness of the HAZ, especially of the fusion line, in such a strong structural steel also at unusually low temperatures.

Moreover, the steel is also excellently weather-resistant, wherein it can also be used when a steel surface patinating to dark brown is a design goal. A steel according to the invention is capable of slowing down corrosion progressing under the paint surface, which increases the security of the structure against corrosion, for example, in places, which are difficult to inspect visually or whose coating to prevent corrosion is difficult or impossible. Likewise, structural inspection intervals and intervals between performances of reparative painting can be increased. Moreover, when suitably alloyed, the steel withstands marine conditions longer than normal, even without coating. When coated, the steel withstands excellently even in a relatively strongly corrosive environment, wherein the adhesion of the coating improves and the need to renew the coating is reduced due to a steel according to the invention.

Good security against corrosion and smooth form of the weld seams to prevent fatigue crackings increase the life cycle of the final product to be produced from an ultra high-strength structural steel according to the invention.

The greatest advantages of a method according to the invention are that it enables a structural steel having above said advantages. Due to direct quenching, no separate heating for hardening and hardening need be performed, which means a significant energy savings. Moreover, direct quenching to a low temperature speeds up the throughput of production, when there is no need to wait for the steel product to cool.

### Brief description of the figures

In the following, the present invention is described in more detail with reference to the accompanying figures, in which:
Fig. 1 shows the main steps of the method according to the invention,
Fig. 1 shows a method, which further has tempering,
Fig. 3 shows in more detail the first preferred embodiment of the method according to the invention, and
Fig. 4 shows in more detail the second preferred embodiment of the method according to the invention.

In the figures, a dashed line means that the next step is a preferred, but not imperative, step of the method.

### Description of the reference numbers

| | |
|---|---|
| Alloying | 2 |
| Pre-rolling | 4 |
| Rolling | 5 |
| Direct-quenching | 8 |
| Turning the sheet 90° | 9 |
| Coiling | 10 |
| Tempering | 12 |

### Detailed description of the invention

The composition of an ultra high-strength structural steel according to the invention comprises, as percentages by weight, the elements recited in claim 1.

Table 1 shows examples of the composition of a steel according to the invention, which composition is described in the following in more detail. The table further has a reference composition R1.

**Table 1. Examples. Contents as percentages by weight**

| **steel** | **C** | **Si** | **Mn** | **Al** | **Cr** | **Ni** | **Cu** | **Mo** | **B** | **Ti** | **Nb** | **V** | **CEV** |
|---|---|---|---|---|---|---|---|---|---|---|---|---|---|
| 1372 | 0.10 | 0.2 | 1.1 | 0.04 | 1.1 | 3.6 | 0.4 | 0.15 | | 0.012 | | | 0.8 |
| 1371 | 0.10 | 0.2 | 1.1 | 0.04 | 1.1 | 1.6 | 2.4 | 0.15 | | 0.012 | | | 0.8 |
| 1370 | 0.10 | 0.2 | 1.1 | 0.04 | 1.5 | 1.6 | 2.4 | 0.60 | | 0.012 | | | 1.0 |
| 1369 | 0.11 | 0.6 | 1.4 | 0.04 | 1.5 | 3.6 | 2.4 | 0.60 | | 0.012 | | | 1.2 |
| R1 | 0.14 | 0.2 | 1.1 | 0.03 | 0.7 | 0.05 | | 0.20 | 0.0019 | 0.031 | 0.003 | 0.009 | 0.5 |

### Carbon C

In relation to its strength level, the steel has a somewhat low carbon content C: 0.07 - 0.12 %, which is useful for the impact toughness and weldability of the material, wherein the carbon equivalent CEV itself can be somewhat high. Carbon C is needed at least 0.07 %, in order that hardening be succeed and ultra-high strength be provided. Preferably, the carbon content C of the steel is 0.08 - 0.12 %, which further improves said properties. Most preferably, the carbon content is in the range of 0.08 - 0.10 %. A low carbon content also hampers the formation of retained austenite between the martensite laths, wherein the risk of hydrogen crackings is reduced.

Surprisingly, a somewhat high carbon equivalent CEV = (C + Mn/6 + (Cr + Mo + V)/5 + (Ni + Cu)/15) in an ultra high-strength structural steel according to the invention influences positively on the providing a combination of good impact toughness and strength in a weld. From Table 1, it is observed that, for an example steel according to the invention, the carbon equivalent CEV > 0.50. Thus, during welding, the re-austenitized zone hardens adequately, wherein it is achieved high strength combined with good impact toughness. More preferably, the carbon equivalent of the steel is 0.5 < CEV < 1.2, most preferably 0.65 < CEV < 1.00.

### Silicon Si

The Si-content of the steel is 0.1 - 0.7 %, especially to achieve strength. Si-contents of less than 0.1 % are not used, because desulphurization and form control of inclusions of the steel is easier, when the steel contains a little silicon. Moreover, silicon Si contributes to improving the weather resistance of a steel. On the other hand, an excessive Si-content can weaken impact strength and impair surface quality. For this reason, Si-content is preferably 0.15 - 0.4 % and most preferably 0.15 - 0.25 %, wherein the excellent surface quality as well as the excellent impact toughness of a sheet-like steel are assured.

### Manganese Mn

The Mn-content of the steel is 0.5 - 2.0 %, because, with manganese, the hardenability of the steel is increased. However, the Mn-content of the steel is preferably moderate, because manganese Mn can infiltrate in continuous casting and can weaken unfavourably the elongation of a direct quenched steel as well as weaken also fracture toughness. For this reason, at the thicknesses of structural steel, manganese is used preferably 0.5 - 1.5 %. According to one preferred embodiment, manganese Mn is alloyed at least 0.7 %, especially when the thickness of the structural steel Tₕ · 5 mm. According to the most preferable embodiment, manganese is alloyed at least 0.9 %, especially when the thickness of the structural steel Tₕ · 6 mm.

### Nickel Ni

The Ni-content of the steel is 0.8 - 4.5 %; preferably 1.5 % - 4.5 %, which is a high content in comparison to a typical structural steel of this strength class. However, by a high Ni-content, it is achieved above all high strength due to increased hardenability without significant risk of hydrogen cracking, wherein the need for preheating during welding can be reduced. Moreover, better impact toughness both of the base metal and of the HAZ is achieved, when it is desired to keep the strength level high in both. Moreover, nickel Ni enables excellent weather resistance properties, which, at contents according to the invention, improve the resistance of the steel even to saltwater corrosion. For this reason, the Ni-content of the steel is most preferably 2.6 - 4.0 %, wherein, for the steel, an excellent saltwater resistance is achieved.

### Copper Cu

In the manner of nickel Ni, the Cu-content of the steel increases the strength of the steel. Moreover, copper Cu increases especially the weather resistance of the steel and it is used 0.25 - 3.0 %. In the invention, the low carbon content of the ultra high-strength steel is made possible especially by alloying Cu and Ni, which is preferable for the weldability.

The combined content of copper Cu and nickel Ni is, as percentages by weight, preferably but not necessarily, at least 2.5 %, according to the following condition Cu(%) + Ni(%) ≥ 2.5 %. In this case, for the steel, high strength at a low carbon content is achieved, which assures good weldability and the achievement of a combination of excellent impact toughness as well as strength in the HAZ of a weld. Preferably, Cu(%)+Ni(%) ≥ 3.0 %, more preferably Cu(%)+Ni(%) ≥ 3.5 %. However, the sum of nickel and copper is preferably not more than 6 %.

Preferably, Cu-content is 2 - 3 %, wherein, for a weld seam provided in a steel according to the invention, high strength and impact toughness is provided. In this case, especially Ni-content can be kept lower, such as Ni 0.8 - 2 %.

According to one embodiment, Cu-content is 0.25 - 2 %, wherein, at reasonable carbon and nickel contents, good weldability and strength properties in relation to the strength properties of the steel are achieved at reasonable alloying element expenses.

### Chromium Cr

The Cr-content of the steel is 0.5 - 1.6 %. Chromium is alloyed at least 0.5 %, because chromium Cr increases the hardenability and strength of the steel and improves the weather resistance. However, an excessively high Cr-content is unnecessary to assure hardenability, when the steel is according to the invention on the part of the other alloying elements. Preferably, Cr-content is 0.7 -1.6 %, most preferably 0.9 - 1.4 %, wherein especially the excellent weather resistance properties of the steel are assured.

For i.a. the weather resistance of the steel, exceptionally essential alloying elements of a structural steel according to the invention are nickel Ni, copper Cu, chromium Cr and silicon Si. To assure weather resistance, the sum content of these alloying elements, as percentages by weight, is preferably at least 3.0 %, i.e. $Cu \left(%\right) + Cr \left(%\right) + Ni \left(%\right) + Si \left(%\right) \geq 3.0 ⁢ %$

Preferably, to assure hardenability, the sum content of chromium Cr and manganese Mn, as percentages by weight, is at least 1.8, i.e. $Mn \left(%\right) + Cr \left(%\right) \geq 1.8 ⁢ %$

### Molybdenum Mo

The Mo-content of the steel is < 0.8 %, because molybdenum Mo increases the strength of steel but, at excessively high contents, it can weaken the cold working properties of a structural steel according to the invention, such as flangeability and, in addition, Mo increases alloying element expenses. Preferably, Mo-content is 0.1-0.8 %, because molybdenum increases the strength and impact toughness by efficiently preventing recrystallization during hot-rolling, wherein austenite grains are flattened and a fine-grained direct quenched microstructure is provided.

Most preferably, Mo-content is 0.1 - 0.25 %, because at least 0.1 % can be needed for the sake of strength, but, on the other hand, Mo-contents of less than 0.25 % contribute to the flangeability of steel.

### Titanium Ti

The Ti-content of the steel is limited Ti ≤ 0.04 %, because high Ti-contents can hinder the success of direct quenching and increase the amount of rough titanium nitrides (TiN) in the steel, which can be of detrimental influence on i.a. impact toughness, fracture toughness and elongation. However, titanium Ti is preferably alloyed at least 0.005 %, because titanium Ti improves the welding properties of the steel by hindering the growth of grains in the HAZ area, wherein a higher heat input can be used, which provides a smooth junction point of the weld bead and the base metal. As a result, due to a small alloying of Ti (0.005 - 0.04 %), weld seams become as impact tough as possible, and from a structural steel according to the invention can be produced by welding exceptionally reliable structures, and also the efficiency of welding work can be increased.

Preferably, Ti-content is ≤ 0.02 %, particularly at greater thicknesses Th ≥ 5 mm, to assure the impact toughness. Most preferably, titanium Ti is thus alloyed 0.005 - 0.02 %.

### Aluminium Al

Aluminium Al can be used to condense the steel at contents of 0.01 - 0.15%. A structural steel according to the invention can achieve excellent resistance welding properties, when Al-content is Al ≤ 0.045 %

### Calcium Ca

Calcium can be used typically 0.0005 - 0.005 %, for example, for the removal of the detrimental influence of the compounds created in connection with desulphurization and/or in condensing.

Preferably, an ultra high-strength structural steel according to the invention consists of only said elements, the rest being iron, and unavoidable impurities.

Unavoidable impurities can be, for example, nitrogen N, phosphorus P and sulphur S. The content of nitrogen N is limited N: ≤ 0.01 %, preferably N: ≤ 0.005 %. A low nitrogen content also makes it possible to keep the level of Ti low.

Due to their detrimental properties, an attempt is made to keep the contents of phosphorus P and sulphur S as small as possible, for example, such that P < 0.02 % and S < 0.04 %. Preferably, S-content is < 0.005 % to provide the best flangeability and impact toughness. However, although a high content of phosphorus P could be of advantage due to weather resistance properties, its influence in weakening impact toughness is so dramatic in such a strong steel, that it cannot be purposely alloyed and contents as low as possible are desirable.

It is unnecessary to alloy vanadium V into a structural steel according to the invention, because, in a structural steel according to the invention, it can weaken the impact toughness and weldability, especially in multi-run welding. Due to that said, the content of vanadium V is, preferably but not necessarily, limited V < 0.1 %, most preferably V ≤ 0.05 %.

Niobium Nb can, in some cases, be alloyed 0.008 - 0.08 % to increase the toughness. However, the use of niobium is not imperative. Preferably, when the ultra high-strength structural steel is a strip steel, i.e. a steel product produced on a strip rolling line, niobium Nb is not alloyed to assure flangeability properties, wherein its content is less than 0.008 %, most preferably less than 0.005 %.

It is unnecessary to alloy Boron B into a structural steel according to the invention, because adequate hardenability is achieved by other alloying elements. Moreover, leaving out alloying of boron enables lowering of the Ti-level to a level according to the invention, because titanium does not need to be alloyed in an amount adequate to assure the function of the boron. Preferably, the boron content of the steel is thus less than 0.0003 %.

However, especially at greater thicknesses Th 9 - 40 mm, boron B can be alloyed 0.0005 - 0.003 %, if hardenability cannot be adequately assured without it. However, in this case, the Ti-content of the steel must be in the range of 0.02 - 0.04 % or such that Ti (%)>3*N(%) but however, Ti ≤ 0.04 %.

The composition of the steel provided in the alloying step 2 makes the steel hardenable, wherein, in direct quenching 8, the steel hardens substantially as martensite. The microstructure of a steel product according to the invention can also consist of self-tempered martensite. There is more than 80 %, preferably more than 90 %, as percentages by volume, of martensite and/or self-tempered martensite. The rest of the microstructure can comprise small amounts of bainite structures, such as upper- or lower bainite.

According to the preferred embodiment, the flatness (aspect ratio) of the prior austenite structure of an ultra high-strength structural steel according to the invention is at least 1.5 and the MLI (mean linear intercept) of the prior austenite structure is less than 20 micrometres.

The definition of MLI is based on the cube root of the product of the cross-section of the three different main directions of prior austenite grain structure. Calculation of the MLI and flatness of the prior austenite structure is described in more detail, for example, in the source: *"*Worked Examples on Quantitative Metallography, The institute of materials, Minerals and Mining, London, UK (2003), p1, ISBN 978 1 902653 80 8*."*

Further, it is typical of a steel product according to the invention that flatness (aspect ratio) and preferably also MLI (mean linear intercept), as measured from different sites of the steel product, are substantially of the same value, which is typical for a hot-rolled product unlike, for example, a steel product having hot-forged shapes. In other words, the deviation of these quantities is low in a steel product according to the invention. As a result, the properties of the steel product are uniform in different points.

According to one embodiment, the steel has been tempered 12 after direct quenching, wherein the steel is tempered martensitic. In this embodiment, it is exceptionally important to alloy copper Cu into the steel, which precipitates during tempering, increasing the strength of the steel.

In a method according to the invention, according to Fig. 1, a steel slab is rolled 5 in a mill such that, at the last pass, the rolling temperature of the steel is 720 - 950 °C, in which method, after the last pass performed in the mill, the steel is direct quenched (8) at a cooling speed of 20 - 150 °C/s to a temperature of not more than 450 °C.

In the following is described the steps of a method according to the invention:
Alloying 2 of the steel is performed by known manners of adding alloying elements, for example, in the steel handling station of CAS-OB. The alloying elements to be added to the steel and their contents are, for the invention, the most substantial matter of method step 2. In this step, the steel is alloyed 2 such that the composition of the steel comprises, as percentages by weight,the elements recited in claim 11.

Thereafter, the steel is continuously cast in a known manner as a steel slab, which is further transferred, for example, after austenitizing annealing (900 - 1350 °C) occurring in a walking beam furnace, to be hot-rolled, in which hot-rolling step 5 the steel slab is rolled to the desired thickness as a sheet-like steel product and direct quenched 8 immediately after rolling 5. In other words, after the last pass of rolling 5, direct quenching 8 is performed.

Specifically when in need of great elongation, tempering 12 can be done for the steel, in which the steel is heated and, thereafter, allowed to cool. Tempering can be done, for example, in the temperature range of 500 - 600 °C typically for approximately 0.2 - 2 hours. At higher temperatures, a shorter tempering time can be used. The highest tempering temperature is 700 °C, because an ultra high-strength structural steel according to the invention is very difficult to achieve above this temperature, even using a very short tempering temperature.

Preferably, processing of the steel is, however, merely thermo-mechanical, wherein, after direct quenching 8, no heat treatments are performed afterwards, such as tempering 12. By the method, steel products can be produced, whose mechanical properties are good without needing to perform on the product an expense-increasing post-welding heat treatment. Tempering 12 is not imperative to improve the mechanical properties of a structural steel according to the invention, because, according to the invention, a tough martensite is achieved. Further, the yield ratio of the structural steel can rise with tempering too close to the value 1, which can be disadvantageous in some applications.

The advantage of a steel direct quenched 8 immediately from hot-rolling is that the alloying elements increasing hardenability are well dissolved and thus efficiently increasing hardenability, because austenitizing annealing has occurred at a high (1000 - 1350 °C) temperature. The grain size of the steel increases at a high reheating temperature, but, in hot-rolling 5, grain size can once again be ground fine through repeated recrystallization of the grain structure. When hot-rolling 5 is continued below the temperature of recrystallization, the austenite can be made to flatten even more, wherein the package size of the martensite decreases and the dislocation density of the martensite rises. In this case, the impact toughness of the martensite formed increases and especially the yield strength increases. Thus, also tensile strengthand hardness can increase slightly. The result is the tough martensitic microstructure of an ultra high-strength structural steel according to the invention.

The present invention enables a tough structure also in a weld joint provided in the steel.

In traditional oven hardening, austenitizing annealing cannot be performed at as high a temperature due to grain growth, because the grain size of the austenite would remain large and the lath package size of the martensite formed as large, which would again weaken the impact toughness of the base metal.

Preferably, with an ultra high-strength structural steel according to the invention to be produced by direct quenching 8, greater strength is achieved at the same chemical composition in comparison to steel produced traditionally by oven hardening. This means that, by a method according to the invention, the amount and contents of the alloying elements can be decreased, which again enables reduction of alloying element expenses.

According to the first embodiment of the method, the structural steel is produced as a strip steel, the specific steps of which, for an invention according to the first embodiment, are shown in Fig. 3.

Fig. 3 shows in more detail the production of an ultra high-strength strip steel according to the first embodiment. After the alloying step 2 and austenitizing annealing (1200 - 1350 °C), the steel slab is rolled according to step 4 of Fig. 3. Rolling 4 is performed, for example, such that, in step 4, hot-rolling is performed at a temperature of 950 - 1280 °C to a thickness of typically 25 - 50 mm, from which it is immediately transferred to the strip mill of step 5, in which it is rolled as a strip, the end thickness of which is 4 - 12 mm. According to recommendations, the end thickness of the strip steel is at least 5 mm. It is also recommended that the end thickness is not more than 10 mm.

The number of passes in the strip mill is typically 5 - 7. The last pass in the strip mill is performed in the temperature range of 760 - 950 °C, according to recommendations in the temperature range of 850 - 920 °C, especially if the strip is relatively thin, wherein the rolling forces remain lower.

After the last pass of rolling 5, direct quenching 8 of the strip steel is begun within 15 seconds. As direct quenching 8 begins, the temperature of the strip steel should be at least 700 °C. Direct-quenching 8 is performed as water quenching such that the speed of quenching is 30 - 150 °C/s, according to recommendations, the upper limit is not more than 120 °C/s. Direct-quenching 8 is performed to a temperature of not more than 300 °C, according to recommendations not more than 100 °C. Immediately after direct quenching 8, the strip steel can be reeled in step 10. The temperature of coiling can then occur in the temperature range of 30 - 300 °C. According to recommendations, the start temperature of coiling 10 is not more than 100 °C, because, when coiling a steel at a temperature of more than 100 °C, a discontinuous cushion of steam can form on the surface of the steel, which complicates the process and causes i.e. weakening of flatness.

Preferably, the end temperature of direct quenching 8 is not more than 100 °C, because, in this case, after quenching, a flat strip is obtained, in which the edges are also even and flat.

Preferably, the steel is direct quenched 8 directly to the ambient temperature.

If needed, tempering treatment 12 can be done to the steel, in which the steel is heated and, thereafter, allowed to cool. Tempering 12 can be done, for example, in the temperature range of 500 - 600 °C, for example, for approximately less than two hours.

For example, a solution implemented with expedited heating is also conceivable, in which possible tempering 12 is performed before coiling 10.

According to the second embodiment of the method, the ultra high-strength structural steel is produced as a steel sheet, more specifically a so-called quarto plate, wherein the essential steps for the second embodiment are shown in Fig. 4.

After the alloying step 2 and austenitizing annealing (1000 - 1300 °C), the steel slab is rolled according to step 5 of Fig. 4. Rolling of the sheet is performed, for example, in a so-called reversible four mill, in which the steel slab is rolled between the mills in back and forth motions at a temperature of 750 - 1300 °C. In step 5, the sheet is rolled either partially or entirely to its final width and, thereafter, a 90° turn 9 is performed in the plane of the sheet. Next, rolling 5 is continued until the desired thickness is achieved. Alternatively, the turn 9 can be performed more than once between the rolling steps 5 and the rolling can be performed in different directions more than once. For the invention, it is essential that, at the last pass of rolling, the temperature in the sheet rolling is less than 950 °C, according to recommendations less than 900 °C. After the last pass of rolling 5, direct quenching 8 of the steel sheet is begun within 30 seconds, preferably within 15 seconds. As direct quenching 8 begins, the temperature of the steel sheet should be at least 700 °C. Direct-quenching 8 is performed as water quenching such that the speed of quenching is 20 - 150 °C/s. Direct-quenching 8 is performed to a temperature of not more than 450 °C, according to recommendations not more than 200 °C.

According to one embodiment, into a structural steel, which is produced in the hot-rolling step of the invention as a steel sheet, is alloyed niobium Nb 0.008 - 0.08 % to increase the toughness.

By a sheet-like steel product is meant such a steel product, whose length and width are noticeably greater than the thickness of rolling, i.e. in other words, by a sheet-like steel product is meant a steel sheet or strip steel. Let it be exemplarily said that the width of a sheet-like steel product can be 1500 mm, while its thickness is 5 mm.

Preferably, the sheet-like steel product is a strip steel, because by strip rolling are achieved the lowest production expenses and the grain structure of the steel can quickly and efficiently be ground fine while hot-rolling 5.

The thickness of an ultra high-strength structural steel according to the invention, Th, is at least 2 mm and preferably at least 4 mm. In the case of strip steels, thickness is preferably Th = 5 - 12 mm, and most preferably Th = 6 - 10 mm, wherein the good impact toughness of the steel is well-utilized in the dimensioning of practical structures and the strip steel is still technically easy to reel as a steel reel.

In the case of quarto plate, the thickness of the steel product can be even 10 - 40 mm, wherein, even at a 40 mm thickness, an adequate depth of hardening according to the invention is achieved. Preferably, the thickness of quarto plate is 12 - 30 mm. If flattened grain structure is, in this case, a specific goal, it is preferable to alloy niobium Nb: 0.008 - 0.08 %.

### Examples

In the following, the invention is illustrated by means of examples made in a laboratory.

55 mm thick miniature meltings according to that shown in Table 1 1372, 1371, 1370, and 1369 were rolled 5 to a thickness of 6 mm using a series of six rolling passes. The slabs were heated in an oven to a temperature of 1225 °C. After the last pass, direct quenching was performed on the sheets. The final dimensions of the rolled steel were 1120x95x6 mm. Tensile test results are shown in accompanying Table 2.

Welding tests were performed using a MAG butt weld as a two-run weld to the groove without root face, in which the groove angle was 50 degrees, root face 0.5 mm and air gap 1.5 mm. The heat input used was, in both the first and the second run welding, approximately 0.6 kJ/mm. In welding, MAG solid wire was used, which is classed as G 89 5 M Mn4Ni2,5CrMo according to the standard EN 12534 and ER120S-G according to standard AWS A 5.28. The weld seams were in the same direction with the rolling direction. The Charpy V impact toughness of the welds was tested using 5X10 mm test bars transverse in relation to the weld seam, and the results are shown in Table 2. The results of the welding tests are comparable when welding is performed according to above said welding test arrangement.

The fusion line FL means the midpoint of the weld joint in the plane of the sheet in the transverse direction in relation to the longitudinal direction of the weld seam. The coarse grained heat affected zone CGHAZ of welding is defined from the site FL+1 mm and ICHAZ from the site FL+3 mm.

The table presents as a reference a full-scale test R1, which is implemented thermo-mechanically by hot-rolling to a thickness of 6 mm and by direct quenching.

As is known, the properties of steels provided in the full scale are higher on the part of strength and impact toughness than the steel properties provided in the laboratory tests, due to the greater degree of deformation and the smaller grain size of prior austenite in the full scale resulting from this. Hence, the properties of a steel product according to the invention are, on an industrial scale, presumably even better than has been demonstrated in this connection. Instead, on the properties of the weld joint in the HAZ this does not have any real influence.

**Table 2. Example tests**

| | **STEEL** | | | | | | **WELD** | | | | | | | | |
|---|---|---|---|---|---|---|---|---|---|---|---|---|---|---|---|
| | | | | | | | Across the weld seam (T) | | | FL | CGHAZ | ICHAZ | FL | CGHAZ | ICHAZ |
| Composition | Rp0.2 (MPa) | Rm (MPa) | Rp0.2 / Rm | A5 (%) | CV -40°C L (J/cm2) | CV -40°C T (J/cm2) | Rp0.2 (MPa) | Rm (MPa) | A5 (%) | CV -40°C T (J/cm2) | CV -40°C T (J/cm2) | CV -40°C T (J/cm2) | CV -60°C T (J/cm2) | CV -60°C T (J/cm2) | CV -60°C T (J/cm2) |
| 1372 | 957 | 1259 | 0.76 | 11.7 | 90 | 44 | 1035 | 1183 | 4,5 | 44 | 50 | 50 | 42 | 48 | 52 |
| 1371 | 968 | 1274 | 0.76 | 12.5 | 108 | 50 | 1045 | 1210 | 5,8 | 50 | 52 | 52 | 38 | 52 | 52 |
| 1370 | 1003 | 1316 | 0.76 | 10.1 | 75 | 40 | - | - | - | - | - | - | - | - | - |
| 1369 | 1035 | 1393 | 0.74 | 11.8 | 69 | 36 | - | - | - | - | - | - | - | - | - |
| R1 | 1102 | 1279 | 0.86 | 11.7 | - | 44 | 932 | 1023 | 3,3 | 22 | 40 | - | - | - | - |

| | | | | | | | | | | | | | | | |
|---|---|---|---|---|---|---|---|---|---|---|---|---|---|---|---|
| FL=fusion line CG HAZ=coarce grained heat affected zone ICHAZ=inter critical heat affected zone CV=Charpy V L=Longitudinal in the rolling direction | | | | | | | | | | | | | | | |

From Table 2, it is observed that, in examples 1372 and 1371, an ultra high-strength steel is achieved, whose impact toughness of the HAZ, as measured transversely in relation to the rolling direction at a temperature of - 40°C, is more than 34 J/ cm², i.e. expressed differently $Charpy V - 40 ° C T \left(FL, ICHAZ, CGHAZ\right) > 34 J / {cm}^{2}$

From Table 2, it is also observed that, in examples 1372 and 1371, an ultra high-strength steel is achieved, whose impact toughness of the coarse grained heat affected zone of the weld, as measured transversely in the rolling direction at a temperature of -40°C, is more than 40 J/ cm², i.e. expressed differently $Charpy V - 40 ° C T \left(CGHAZ\right) > 40 J / {cm}^{2} .$

From Table 2, it is also observed that, in examples 1372 and 1371, an ultra high-strength steel is achieved, whose impact toughness of the heat affected zone of the weld, as measured from the fusion line transversely in the rolling direction at a temperature of -40°C, is more than 35 J/ cm², i.e. expressed differently $Charpy V - 40 ° C T \left(FL\right) > 35 J / {cm}^{2} .$

Preferably, a steel according to the invention meets corresponding impact toughness requirements also at a temperature of -60 °C.

From Table 2, it is observed especially that the ultra high-strength structural steel R1, which belongs outside of the invention, is more fragile in the heat affected zone of the weld than ultra high-strength steels 1372 and 1371 according to the invention.

Further, from Table 2, it is observed that, in example 1372, an ultra high-strength steel is achieved, whose yield strength Rₚ₀.₂ is approximately 957 MPa and Charpy V -40 °C > 50 J/cm², as measured longitudinally in relation to the rolling direction. Making reference to that said earlier, by doing the same on an industrial scale, a yield strength of at least 960 MPa can assuredly be achieved.

Further, from Table 2, it is observed that, in the examples, the yield strength R_{p0.2} of the HAZ is at least as great as the yield strength R_{p0.2} of the base metal. On an industrial scale, the yield strength R_{p0.2} of the HAZ can be achieved substantially as great as the yield strength of the base metal R_{p0.2}, such as that the yield strength R_{p0.2} of the HAZ is at least 85%, preferably at least 90% of the yield strength R_{p0.2} of the base metal or greater.

Further, from Table 2, it is observed that, in example 1371, an ultra high-strength steel is achieved, whose yield strength R_{p0.2} is at least 960 MPa and Charpy V of the base metal -40 °C > 50 J/cm², as measured longitudinally in relation to the rolling direction.

By the invention, a structural steel can be provided having the following superior mechanical properties:
- yield strength R_{p0.2} = 960 - 1250 MPa. Such as even R_{p0.2} = 1100 - 1250 MPa. *
- tensile strengthRₘ 980 - 1500 MPa. Such as even 1120 - 1500 MPa *
- yield ratio (R_{p0.2}/ Rₘ) > 0.7. Such as (R_{p0.2}/ Rₘ) > 0.8. *
- elongation at break A₅ > 7 %. Such as even A5 > 8 %. *
- when tempering heat-treated 12, elongation at break A₅ > 8 %. Such as even A₅ > 10%. *
- impact toughness of the base metal Charpy V -20 °C > 50 J/cm²,
   Such as even Charpy V -40 °C > 50 J/ cm²
   Such as especially even Charpy V -60 °C > 50 J/ cm². * **
      * *as measured by a rod longitudinal in relation to the rolling direction.*
      ** *is measured by a rod having the thickness of the sheet, but by a max. 10 mm rod*

When welding an ultra high-strength structural steel according to the invention, welding methods typically used in welding high-strength steels can be used without problems and welding can be done from ultra-high strength, without problems, by the normal heat inputs used in welding high-strength steels. Naturally, extremely great welding energies attempt to lower the strength of the weld joint somewhat in relation to the small energies. A steel suitably Ti-alloyed according to the invention is capable of well resisting grain growth in the heat affected zone (HAZ) created during welding, which has an advantageous influence on the impact toughness of the so-called coarse grained zone. Moreover, a structural steel according to the invention hardens efficiently during welding over the re-austenitized zone, wherein the strength of the weld is made high. Due to advantageous grain size of the zone and martensite created due to low carbon content, impact toughness properties are exceptionally good for such a strong structural steel, even though the carbon equivalent is somewhat high. In multi-run welding are also achieved good toughness and strength properties due to a suitable composition, for example, by limiting vanadium content. Preferably, also in welding done in an orthodox manner, yield strength of the weld to be achieved in a transverse tensile test across the weld seam is at least 960 MPa, such as has been demonstrated above.

Moreover, the fracture toughness behaviour of a structural steel produced by the method according to the invention is preferred i.a. due to its low C-content and high Ni-content, i.e. the energy needed for the distortion nucleation and progression is great considering the strength and production manner of the steel and steel fractures persistently especially in the direct quenched 8 state. This is an especially preferred and often imperative property for such a strong structural steel. The property can be roughly evaluated through impact toughness, which, in an ultra high-strength structural steel produced by a method according to the invention, is excellent.

The invention is described in the above by means of the preferred embodiments and it is obvious that the invention can be implemented in its details in many different ways within the scope of the accompanying claims.

## Claims

1. A hot-rolled ultra high-strength structural steel, whose yield strength R_{p0.2} is at least 960 MPa, wherein the microstructure of the structural steel is, as percentage by volume, more than 80% martensitic and/or self-tempered martensitic, ***characterized in that*** the composition of the structural steel comprises, as percentages by weight:
C: 0.07 - 0.12 %,
Si: 0.1 - 0.7 %,
Mn: 0.5 - 2.0 %,
Ni: 0.8 - 4.5 %,
Cu: 0.25 - 3.0 %,
Cr: 0.5 - 1.6 %,
Mo: 0.1 - 0.8 %,
Ti: 0.005 - 0.04 %
Al: 0.01 - 0.15%
the rest being iron (Fe), unavoidable impurities such as
N≤0.01 %, P<0.02 %, S<0.04 %
and optionally one or more of the following
V: less than 0.1%
B: less than 0.0003 % or B: 0.0005 - 0.003 % combined with Ti (%) higher than 3*N (%) or Ti: 0.02 - 0.04 %
Nb: 0.008 - 0.08 % or less than 0.008 %,
Ca: 0.0005 - 0.005 %,
and **in that** the carbon equivalent CEV of the structural steel, as calculated by the formula CEV= (C + Mn/6 + (Cr + Mo + V)/5 + (Ni + Cu)/15) is in the range of 0.5 - 1.2.

2. A hot-rolled ultra high-strength structural steel according to claim 1, ***characterized in that*** C-content, as percentages by weight, is C: 0.08 - 0.12 %, more preferably 0.08 - 0.10 %.

3. A hot-rolled ultra high-strength structural steel according to claim 1 or *2, **characterized in that*** Ni-content, as percentages by weight, is Ni: 1.5 - 4.5 %, preferably 2.6 - 4.0 %.

4. A hot-rolled ultra high-strength structural steel according to any one of claims 1 - 3, ***characterized in that*** Mo-content, as percentages by weight, is Mo: 0.1 - 0.80 %, preferably 0.1 - 0.25 %.

5. A hot-rolled ultra high-strength structural steel according to any one of claims 1 - 4, ***characterized in that*** Ti-content, as a percentage by weight, is 0.005 - 0.02 %.

6. A hot-rolled ultra high-strength structural steel according to any one of claims 1 - 5, ***characterized in that*** the carbon equivalent CEV of the structural steel, as calculated by the formula CEV = (C + Mn/6 + (Mo + V)/5 + (Ni + Cu)/15), is in the range of 0.65 - 1.0, even most preferably in the range of 0.65 - 0.9 to assure the hardenability of the re-austenitized zone of the weld.

7. A hot-rolled ultra high-strength structural steel according to any one of claims 1 - 6, ***characterized in that*** the flatness (aspect ratio) of the prior austenite grain structure of the ultra high-strength structural steel is at least 1.5 and the MLI (mean linear intercept) of the prior austenite structure less than 20 micrometres.

8. A hot-rolled ultra high-strength structural steel according to any one of claims 1 - 7, ***characterized in that*** the ultra high-strength structural steel is a strip steel, whose thickness Th = 2 - 12 mm, preferably 4 - 12 mm.

9. A hot-rolled ultra high-strength structural steel according to any one of claims 1 - 8, ***characterized in that*** the ultra high-strength structural steel is produced by direct quenching (8) the steel directly from strip rolling (5).

10. A hot-rolled ultra high-strength structural steel according to any one of claims 1 - 9, ***characterized in that*** the impact toughness of the HAZ of a weld provided in the ultra high-strength structural steel, as measured transversely in relation to the rolling direction at a temperature of -40°C, is more than 34 J/ cm².

11. A method for producing an ultra high-strength structural steel, wherein the yield strength R_{p0.2} of the ultra high-strength structural steel is at least 960 MPa, in which method the steel slab is rolled (5) in a mill such that, at the last pass, the rolling temperature of the steel slab is 720 - 950 °C, in which method, after the last pass performed in the mill, the steel slab is direct quenched (8) at a cooling speed of 20 - 150 °C/s to a temperature of not more than 450°C to obtain ultra-high strength structural steel, wherein processing of the steel is merely thermo-mechanical, wherein after direct quenching (8) no heat treatments are performed afterwards, ***characterized in that*** the steel is alloyed (2) for a steel slab such that the composition of the steel comprises, as percentages by weight, the following element contents:
C: 0.07 - 0.12 %,
Si: 0.1 - 0.7 %,
Mn: 0.5 - 2.0 %,
Ni: 0.8 - 4.5 %,
Cu: 0.25 - 3.0 %,
Cr: 0.5 - 1.6 %,
Mo: 0.1 - 0.8 %,
Ti: 0.005 - 0.04 %
Al: 0.01 - 0.15%
the rest being iron (Fe), unavoidable impurities such as
N≤0.01 %, P<0.02 %, S<0.04 %
and optionally one or more of the following
V: less than 0.1%
B: less than 0.0003 % or B: 0.0005 - 0.003 % combined with Ti (%) higher than 3*N(%) or Ti: 0.02 - 0.04 %
Nb: 0.008 - 0.08 % or less than 0.008 %,
Ca: 0.0005 - 0.005 %,
**and in that** the carbon equivalent CEV of the structural steel, as calculated by the formula CEV= (C + Mn/6 + (Cr + Mo + V)/5 + (Ni + Cu)/15) is in the range of 0.5 - 1.2.

12. A method according to claim 11, ***characterized in that*** the steel is alloyed (2) such that C-content, as percentages by weight, is 0.08 - 0.12 %, more preferably 0.08 - 0.10 %.

13. A method according to claim 11 or 12, ***characterized in that*** the steel is alloyed (2) such that Ni-content, as percentages by weight, is Ni: 1.5 - 4.5 %, more preferably 2.6 - 4.0 %.

14. A method according to any one of claims 11 - 13, ***characterized in that*** the steel is alloyed (2) such that Ti-content, as a percentage by weight, is 0.005 - 0.02 %.

15. A method according to any one of claims 11 - 14, ***characterized in that*** the steel is alloyed (2) such that carbon equivalent of the steel, as calculated by the formula CEV = (C + Mn/6 + (Mo + V)/5 + (Ni + Cu)/15), is in the range of 0.65 - 1.0, even most preferably in the range of 0.65 - 0.9 to assure the hardenability of the re-austenitized zone of the weld.

## Patentansprüche

1. Warmgewalzter ultrahochfester Baustahl, dessen Streckgrenze R_{p0,2} mindestens 960 MPa beträgt, wobei die Mikrostruktur des Baustahls in Volumenprozent mehr als 80% martensitisch und/oder selbstvergütet martensitisch beträgt, ***dadurch gekennzeichnet, dass*** die Zusammensetzung des Baustahls in Gewichtsprozent umfasst:
C: 0,07-0,12 %
Si: 0,1-0,7 %,
Mn: 0,5-2,0 %,
Ni: 0,8-4,5 %,
Cu: 0,25-3,0 %
Cr: 0,5-1,6 %
Mo: 0,1-0,8 %,
Ti: 0,005-0,04 %
Al: 0,01-0,15 %
der Rest Eisen (Fe), unvermeidbare Verunreinigungen wie N≤0,01 %, P<0,02 %, S<0,04 %
und gegebenenfalls eines oder mehrere von Folgenden ist
V: weniger als 0,1 %
B: weniger als 0,0003 % oder B: 0,0005-0,003 % kombiniert mit Ti (%) höher als 3^{∗}N (%) oder Ti: 0,02-0,04 %
Nb: 0,008-0,08 % oder weniger als 0,008 %,
Ca: 0,0005-0,005 %,
und dadurch, dass das Kohlenstoffäquivalent CEV des Baustahls, berechnet durch die Formel CEV= (C + Mn/6 + (Cr + Mo + V)/5 + (Ni + Cu)/15) im Bereich von 0,5-1,2 liegt.

2. Warmgewalzter ultrahochfester Baustahl nach Anspruch 1, ***dadurch gekennzeichnet, dass*** der C-Gehalt in Gewichtsprozent, C: 0,08-0,12 %, bevorzugter 0,08-0,10 % beträgt.

3. Warmgewalzter ultrahochfester Baustahl nach Anspruch 1 oder 2, ***dadurch gekennzeichnet, dass*** der Ni-Gehalt in Gewichtsprozent, Ni: 1,5-4,5 %, vorzugsweise 2,6-4,0 % beträgt.

4. Warmgewalzter ultrahochfester Baustahl nach einem der Ansprüche 1-3, ***dadurch gekennzeichnet, dass*** der Mo-Gehalt in Gewichtsprozent, Mo: 0,1-0,80 %, vorzugsweise 0,1-0,25 % beträgt.

5. Warmgewalzter ultrahochfester Baustahl nach einem der Ansprüche 1-4, ***dadurch gekennzeichnet, dass*** der Ti-Gehalt in Gewichtsprozent, 0,005-0,02 % beträgt.

6. Warmgewalzter ultrahochfester Baustahl nach einem der Ansprüche 1-5, ***dadurch gekennzeichnet, dass*** das Kohlenstoffäquivalent CEV des Baustahls, berechnet nach der Formel CEV = (C + Mn/6 + (Mo + V)/5 + (Ni + Cu)/15), im Bereich von 0,65-1,0, sogar besonders bevorzugt im Bereich von 0,65-0,9 liegt, um die Härtbarkeit der neu austenitisierten Zone der Schweißnaht sicherzustellen.

7. Warmgewalzter ultrahochfester Baustahl nach einem der Ansprüche 1-6, ***dadurch gekennzeichnet, dass*** die Flachheit (Seitenverhältnis) der vorherigen Austenitkornstruktur des ultrahochfesten Baustahls mindestens 1,5 und der MLI (mittlerer linearer Achsenabschnitt) der vorherigen Austenitstruktur weniger als 20 Mikrometer beträgt.

8. Warmgewalzter ultrahochfester Baustahl nach einem der Ansprüche 1-7, ***dadurch gekennzeichnet, dass*** der ultrahochfeste Baustahl ein Bandstahl ist, dessen Dicke Th = 2 bis 12 mm, vorzugsweise 4 bis 12 mm beträgt.

9. Warmgewalzter ultrahochfester Baustahl nach einem der Ansprüche 1-8, ***dadurch gekennzeichnet, dass*** der ultrahochfeste Baustahl durch direktes Abschrecken (8) des Stahls direkt aus dem Bandwalzen (5) hergestellt wird.

10. Warmgewalzter ultrahochfester Baustahl nach einem der Ansprüche 1-9, ***dadurch gekennzeichnet, dass*** die Schlagzähigkeit der HAZ einer im ultrahochfesten Baustahl bereitgestellten Schweißnaht, wie quer zur Walzrichtung gemessen, bei einer Temperatur von -40 °C mehr als 34 J/cm² beträgt.

11. Verfahren zur Herstellung eines ultrahochfesten Baustahls, wobei die Streckgrenze R_{p0,2} des ultrahochfesten Baustahls mindestens 960 MPa beträgt, wobei in dem Verfahren die Stahlbramme in einem Walzwerk so gewalzt wird (5), dass beim letzten Durchgang die Walztemperatur der Stahlbramme 720-950 °C beträgt, wobei in dem Verfahren die Stahlbramme nach dem in dem Walzwerk durchgeführten letzten Durchgang direkt mit einer Abkühlgeschwindigkeit von 20-150 °C/s auf eine Temperatur von nicht mehr als 450 °C abgeschreckt wird (8), um ultrahochfesten Baustahl zu erhalten, wobei die Verarbeitung des Stahls rein thermomechanisch ist, wobei nach dem direkten Abschrecken (8) keine Wärmebehandlungen mehr durchgeführt werden, ***dadurch gekennzeichnet, dass*** der Stahl für eine Stahlbramme legiert wird (2), sodass die Zusammensetzung des Stahls in Gewichtsprozent die folgenden Elementgehalte umfasst:
C: 0,07-0,12 %
Si: 0,1-0,7 %,
Mn: 0,5-2,0 %,
Ni: 0,8-4,5 %,
Cu: 0,25-3,0 %
Cr: 0,5-1,6 %
Mo: 0,1-0,8 %,
Ti: 0,005-0,04 %
Al: 0,01-0,15 %
der Rest Eisen (Fe), unvermeidbare Verunreinigungen wie N≤0,01 %, P<0,02 %, S<0,04 %
und gegebenenfalls eines oder mehrere von Folgenden ist
V: weniger als 0,1 %,
B: weniger als 0,0003 % oder B: 0,0005-0,003 % kombiniert mit Ti (%) höher als 3^{∗}N (%) oder Ti: 0,02-0,04 %
Nb: 0,008-0,08 % oder weniger als 0,008 %,
Ca: 0,0005-0,005 %,
**und dadurch, dass** das Kohlenstoffäquivalent CEV des Baustahls, berechnet durch die Formel CEV = (C + Mn/6 + (Cr + Mo + V)/5 + (Ni + Cu)/15) im Bereich von 0,5-1,2 liegt.

12. Verfahren nach Anspruch 11, ***dadurch gekennzeichnet, dass*** der Stahl legiert wird (2), sodass der C-Gehalt in Gewichtsprozent 0,08 bis 0,12 %, bevorzugter 0,08 bis 0,10 % beträgt.

13. Verfahren nach Anspruch 11 oder 12, ***dadurch gekennzeichnet, dass*** der Stahl legiert wird (2), sodass der Ni-Gehalt in Gewichtsprozent Ni: 1,5-4,5 %, bevorzugter 2,6-4,0 % beträgt.

14. Verfahren nach einem der Ansprüche 11-13, ***dadurch gekennzeichnet, dass*** der Stahl legiert wird (2), sodass der Ti-Gehalt in Gewichtsprozent 0,005-0,02 % beträgt.

15. Verfahren nach einem der Ansprüche 11-14, ***dadurch gekennzeichnet, dass*** der Stahl legiert wird (2), sodass das Kohlenstoffäquivalent des Stahls, berechnet nach der Formel CEV = (C + Mn/6 + (Mo + V)/5 + (Ni + Cu)/15), im Bereich von 0,65-1,0, sogar besonders bevorzugt im Bereich von 0,65-0,9 liegt, um die Härtbarkeit der neu austenitisierten Zone der Schweißnaht sicherzustellen.

## Revendications

1. Acier de construction à ultra-haute résistance laminé à chaud, dont la limite d'élasticité R_{p0,2} vaut au moins 960 MPa, dans lequel la microstructure de l'acier de construction est, en pourcentage par volume, à plus de 80 % martensitique et/ou martensitique auto-trempée, ***caractérisé en ce que*** la composition de l'acier de construction comprend, en pourcentages en poids :
C : de 0,07à 0,12%,
Si : de 0,1à 0,7%,
Mn : de 0,5 à 2,0%,
Ni : de 0,8 à 4,5 %,
Cu : de 0,25 à 3,0 %,
Cr : de 0,5 à 1,6 %,
Mo : de 0,1à 0,8%,
Ti : de 0,005 à 0,04 %,
Al : de 0,01 à 0,15 %,
le reste étant du fer (Fe), des impuretés inévitables telles que N ≤ 0,01%, P < 0,02 %, S < 0,04 %,
et facultativement l'un ou plusieurs des suivants
V : moins de 0,1 %,
B : moins de 0,0003 % ou B : de 0,0005 à 0,003 % combiné avec Ti (%) supérieur à 3^{∗}N (%) ou Ti : de 0,02 à 0,04 %,
Nb : de 0,008 à 0,08 % ou moins de 0,008 %,
Ca : de 0,0005 à 0,005 %,
et **en ce que** l'équivalent carbone CEV de l'acier de construction, comme calculé par la formule CEV = (C + Mn/6 + (Cr + Mo + V)/5 + (Ni + Cu)/15), est dans la gamme de 0,5 à 1,2.

2. Acier de construction à ultra-haute résistance laminé à chaud selon la revendication 1, ***caractérisé en ce que*** la teneur en C, en pourcentages en poids, vaut C : de 0,08 à 0,12 %, plus préférentiellement de 0,08 à 0,10 %.

3. Acier de construction à ultra-haute résistance laminé à chaud selon la revendication 1 ou 2, ***caractérisé en ce que*** la teneur en Ni, en pourcentages en poids, vaut Ni : de 1,5 à 4,5 %, de préférence de 2,6 à 4,0 %.

4. Acier de construction à ultra-haute résistance laminé à chaud selon l'une quelconque des revendications 1 à 3, ***caractérisé en ce que*** la teneur en Mo, en pourcentages en poids, vaut Mo : de 0,1 à 0,80 %, de préférence de 0,1 à 0,25 %.

5. Acier de construction à ultra-haute résistance laminé à chaud selon l'une quelconque des revendications 1 à 4, ***caractérisé en ce que*** la teneur en Ti, en pourcentage en poids, vaut de 0,005 à 0,02 %.

6. Acier de construction à ultra-haute résistance laminé à chaud selon l'une quelconque des revendications 1 à 5, ***caractérisé en ce que*** l'équivalent carbone CEV de l'acier de construction, comme calculé par la formule CEV = (C + Mn/6 + (Mo + V)/5 + (Ni + Cu)/15), est dans la gamme de 0,65 à 1,0, même le plus préférentiellement dans la gamme de 0,65 à 0,9 pour assurer la trempabilité de la zone ré-austénisée de la soudure.

7. Acier de construction à ultra-haute résistance laminé à chaud selon l'une quelconque des revendications 1 à 6, ***caractérisé en ce que*** la planéité (rapport hauteur/largeur) de la structure de départ à grains d'austénite de l'acier de construction à ultra-haute résistance vaut au moins 1,5 et l'IML (interception moyenne linéaire) de la structure de départ d'austénite est inférieure à 20 micromètres.

8. Acier de construction à ultra-haute résistance laminé à chaud selon l'une quelconque des revendications 1 à 7, ***caractérisé en ce que*** l'acier de construction à ultra-haute résistance est un feuillard d'acier, dont l'épaisseur Th vaut de 2 à 12 mm, de préférence de 4 à 12 mm.

9. Acier de construction à ultra-haute résistance laminé à chaud selon l'une quelconque des revendications 1 à 8, ***caractérisé en ce que*** l'acier de construction à ultra-haute résistance est produit par trempage direct (8) de l'acier directement depuis le laminage à feuillard (5).

10. Acier de construction à ultra-haute résistance laminé à chaud selon l'une quelconque des revendications 1 à 9, ***caractérisé en ce que*** la résistance aux chocs de l'HAZ d'une soudure fournie dans l'acier de construction à ultra-haute résistance, telle que mesurée transversalement par rapport au sens de laminage à une température de - 40 °C, vaut plus que 34 J/cm².

11. Procédé de production d'un acier de construction à ultra-haute résistance, dans lequel la limite d'élasticité R_{p0,2} de l'acier de construction à ultra-haute résistance vaut au moins 960 MPa, dans lequel la brame d'acier est laminée (5) dans un laminoir de sorte que, à la dernière passe, la température de laminage de la brame d'acier est entre 720 et 950 °C, dans lequel, après la dernière passe exécutée dans le laminoir, la brame d'acier est trempée directement (8) à une vitesse de refroidissement d'entre 20 et 150 °C/s à une température ne dépassant pas 450 °C pour obtenir de l'acier de construction à ultra-haute résistance, dans lequel le traitement de l'acier est simplement thermomécanique, dans lequel, après le trempage direct (8), aucun traitement thermique n'est effectué ensuite, ***caractérisé en ce que*** l'acier est allié (2) pour une brame d'acier de sorte que la composition de l'acier comprenne, en pourcentages en poids, les teneurs en élément suivantes :
C :de 0,07à 0,12 %,
Si : de 0,1à 0,7 %,
Mn : de 0,5 à 2,0 %,
Ni : de 0,8 à 4,5 %,
Cu : de 0,25 à 3,0 %,
Cr : de 0,5 à 1,6 %,
Mo: de 0,1à 0,8 %,
Ti : de 0,005 à 0,04 %,
Al : de 0,01 à 0,15 %,
le reste étant du fer (Fe), des impuretés inévitables telles que N ≤ 0,01 %, P < 0,02 %, S < 0,04 %,
et facultativement l'un ou plusieurs des suivants
V : moins de 0,1 %,
B : moins de 0,0003 % ou B : de 0,0005 à 0,003 % combiné avec Ti (%) supérieur à 3^{∗}N (%) ou Ti : de 0,02 à 0,04 %,
Nb : de 0,008 à 0,08 % ou moins de 0,008 %,
Ca : de 0,0005 à 0,005 %,
**et en ce que** l'équivalent carbone CEV de l'acier de construction, comme calculé par la formule CEV = (C + Mn/6 + (Cr + Mo + V)/5 + (Ni + Cu)/15), est dans la gamme de 0,5 à 1,2.

12. Procédé selon la revendication 11, ***caractérisé en ce que*** l'acier est allié (2) de sorte que la teneur en C, en pourcentages en poids, vaut de 0,08 à 0,12 %, plus préférentiellement de 0,08 à 0,10 %.

13. Procédé selon la revendication 11 ou 12, ***caractérisé en ce que*** l'acier est allié (2) de sorte que la teneur en Ni, en pourcentages en poids, vaut Ni : de 1,5 à 4,5 %, plus préférentiellement de 2,6 à 4,0 %.

14. Procédé selon l'une quelconque des revendications 11 à 13, ***caractérisé en ce que*** l'acier est allié (2) de sorte que la teneur en Ti, en pourcentage en poids, vaut de 0,005 à 0,02 %.

15. Procédé selon l'une quelconque des revendications 11 à 14, ***caractérisé en ce que*** l'acier est allié (2) de sorte que l'équivalent carbone de l'acier, comme calculé par la formule CEV = (C + Mn/6 + (Mo + V)/5 + (Ni + Cu)/15), est dans la gamme de 0,65 à 1,0, même le plus préférentiellement dans la gamme de 0,65 à 0,9 pour assurer la trempabilité de la zone ré-austénisée de la soudure.
